

## UNITED STATES PATENT OFFICE

2,243,858

## PRODUCTION OF TEXTILE MATERIALS

Bernard Joseph Flanagan and Albert Mellor,  
Spondon, near Derby, England, assignors to  
Celanese Corporation of America, a corporation  
of Delaware

No Drawing. Application March 29, 1938, Serial  
No. 198,683. In Great Britain April 23, 1937

9 Claims. (Cl. 8—114)

This invention relates to the production of textile materials, and particularly to the production of crêpe fabrics containing highly twisted crêpe yarns having a basis of organic esters of cellulose.

Crêpe fabrics may be obtained by highly twisting yarns of cellulose acetate or other organic ester of cellulose and weaving such yarns into fabric form. Crêpe fabrics of especial value are obtained by forming the fabrics from yarns of cellulose acetate or other organic ester of cellulose which have been highly twisted by a process in which at least the last part of the high twist is inserted while the yarns are under the influence of steam or hot water, processes of this type being described in U. S. Patents Nos. 2,088,628, 2,088,587 and 2,089,191. On treating the fabrics produced by any of these processes with hot aqueous liquids, e. g. hot soap solutions, the fabrics shrink and acquire a crêpe appearance, this crêpe appearance being more pronounced in the case of fabrics containing yarns produced by the processes of the above mentioned specifications. Such treatment with hot aqueous liquids is generally referred to as the "crêping operation" and the liquid used is referred to as the "crêping bath."

In order to obtain the best results the crêping operation must be continued long enough to allow a considerable shrinkage of the high twist yarns to take place. It has now been discovered, however, that the duration of the crêping operation necessary in the case of fabrics containing high twist crêpe yarns of cellulose acetate or other organic esters of cellulose can be considerably reduced whilst effecting at least the same amount of shrinkage or, in other words, that the rate of shrinkage of such high twist crêpe yarns during the crêping operation can be considerably increased, if the fabric containing such high twist crêpe yarns is treated prior to the crêping operation with agents having a hydrolysing or saponifying action on the cellulose ester present. Furthermore, by means of the new process it is possible to obtain satisfactory crêpe effects with the aid of cellulose ester yarns which are twisted to a lower degree than is necessary to obtain similar effects if the hydrolysing treatment is not applied, e. g. 10 to 20 turns per inch less.

The treatment with the hydrolysing or saponifying agent may be such that considerable hydrolysis or saponification is effected, e. g. a loss of 20 to 30% in the weight of the materials. Preferably, however, the saponification or hy-

drosis effected is not so great as to destroy the affinity of the materials for dyestuffs having affinity for cellulose ester materials, and very satisfactory results may be obtained if only a slight saponification or hydrolysis is effected, e. g. a saponification or hydrolysis resulting in a loss of only 1 to 3 or 5% of the weight of the cellulose ester materials.

The fabric treated may be formed entirely of 10 yarns of cellulose acetate or other organic ester of cellulose or may be a mixed fabric containing, in addition to high twist crêpe yarns of cellulose acetate or other organic ester of cellulose, crêpe yarns or other yarns of regenerated cellulose (produced, for example, by the viscose, cuprammonium or nitrocellulose processes) or 15 yarns of cotton, silk or wool. The high twist crêpe yarns of cellulose acetate or other organic ester of cellulose may be contained in the warp or weft of the fabric or both in the warp and in the weft. Particularly valuable results are obtained in the treatment of fabrics which contain cellulose acetate warp yarns of relatively 20 low twist, and in the weft both high twist cellulose acetate crêpe yarns having a left-hand twist and high twist cellulose acetate crêpe yarns having a right-hand twist, pairs of yarns of left-hand twist alternating with pairs of yarns of right-hand twist.

25 The hydrolysing agents used for the treatment of the fabric may be, for example, inorganic acids, e. g. hydrochloric acid, or organic acids, e. g. formic acid and oxalic acid. Preferably, however, strong saponifying agents are employed 30 such as caustic alkalies and alkali metal salts of weak acids, e. g. caustic soda, caustic potash and sodium carbonate.

In general the hydrolysing or saponifying agents are applied to the fabrics in the form of 35 aqueous solutions. The application of the solutions may be effected, for example, by immersing the fabrics in the solutions or by contacting the fabrics with padding rollers supplied with the solutions. The method of applying the solutions to 40 the fabrics is preferably such that the amount of solution carried by the fabrics can be adjusted. Thus the fabrics may be passed through nip rollers adjusted to leave the desired amount of solution in the fabrics.

45 After the treatment of the fabric with the hydrolysing or saponifying agent the fabric is preferably dried, though this is not absolutely necessary. It is found that, in general, not only are greater rates of shrinkage obtained if the treated 50 fabric is dried prior to the crêping operation but

the total amount of shrinkage obtained is greater. The drying may be effected in any convenient manner, e. g. by passing the fabric through a chamber containing hot air or other hot gas, or by passing the fabric in contact with hot surfaces as, for example, heated metal drums. The temperature of drying may vary considerably but it is found that the best results are obtained if the drying is carried out at 50 to 100° C. and preferably 75 to 100° C. The drying of the fabric is preferably effected while the fabric is under the minimum possible tension.

After such a drying operation the fabric is preferably washed with warm water or a warm soap solution, e. g. at a temperature up to 50 15 to 60° C. prior to the crêping operation.

The optimum concentration of the solution of hydrolysing or saponifying agent applied to the fabric varies according to whether the fabric is passed direct from the application of such agent to the crêping bath or is dried, or dried and washed, before being passed to the crêping bath. Thus it is found that very valuable results can be obtained by treating fabric containing high twist crêpe yarns of cellulose acetate with solutions containing 0.5 to 3% of caustic soda, the optimum concentrations where the fabric is passed direct to the crêping operation being about 1.5 to 2.5%, and the optimum concentrations where the fabric is dried prior to the crêping 30 operation being about 1.25 to 1.75%, the amount of caustic soda solution carried by the fabric being in each case about 80% of the weight of the fabric. In the treatment of fabric containing high twist crêpe yarns of cellulose acetate with solutions of sodium carbonate in accordance with this invention, a satisfactory concentration of sodium carbonate appears to be about 2 to 3%, the amount of sodium carbonate solution carried by the fabric being about 80% of the 40 weight of the fabric.

The crêping operation may consist, for example, in a treatment of the fabric with a hot aqueous soap solution, e. g., a treatment with a 0.5% solution of soap at a temperature of at least 45 80° C., and preferably just below boiling temperature. A satisfactory degree of shrinkage can be produced by subjecting fabrics treated in accordance with this invention to treatment for periods of less than one minute in such solutions. Since the steps of treating the fabric with a hydrolysing or saponifying agent, drying the fabric and washing the fabric also take only a very short time to carry out, the whole treatment of the fabric according to the new process can be effected as a continuous operation. Thus the fabric may be passed continuously through a vessel containing a solution of a hydrolysing or saponifying agent, thence between nip rollers to adjust the amount of solution retained by the fabric, thence through a hot chamber or in contact with a heated surface, thence into a washing bath, and finally into the crêping bath.

The following examples illustrate the invention but are not to be regarded as limiting it in any way:

#### Example 1

A cellulose acetate fabric containing cellulose acetate yarns which have been highly twisted by one of the processes of the specifications mentioned above is padded with a 1.5% solution of caustic soda and the amount of solution retained by the fabric adjusted to about 80% of the weight of the fabric. The fabric is then led into a hot air chamber and dried at 75 to 100° C. under

substantially no tension. The fabric is then led through warm water and finally into a 1/2 soap solution maintained at about 99° C. The rate of travel of the fabric is adjusted so that it is in contact with this hot soap solution for a period of half a minute. An excellent crêpe effect is obtained.

#### Example 2

A cellulose acetate fabric containing cellulose acetate yarns which have been highly twisted by one of the processes of the specifications mentioned above is padded with a 2% sodium carbonate solution and the amount of solution retained by the fabric adjusted to about 80% of the weight of the fabric. The fabric is then led into a hot air chamber at 75° C. under minimum tension and is then passed directly into a crêping bath consisting of a 1/2% soap solution maintained at about 99° C. The rate of travel of the fabric is adjusted so that the fabric is in contact with this hot soap solution for half a minute. An excellent crêpe effect is obtained.

When using caustic soda and sodium carbonate in accordance with this invention there is usually a very rapid reduction in the lustre of the fabric as it passes through the crêping bath. This result is apparently due to the fact that some sodium acetate is formed on the fabric, a conclusion which is supported by the fact that by padding the fabric with sodium acetate prior to crêping a very rapid delustring is obtained during the crêping operation. This property of sodium acetate appears to be shared by sodium, ammonium and potassium salts generally, e. g. sodium carbonate, sodium bicarbonate, sodium chloride and sodium nitrite, and also by some metal salts, e. g. barium chloride, and it is not a property which depends entirely on the use of a soap solution as the crêping bath since substitution of a hot water bath produces similar results though generally to a lesser degree.

If it is desired to preserve the lustre of the fabric, some improvement may be effected by adopting the expedient of washing the fabric with warm water prior to the crêping operation. A better method of preserving the lustre, however, is by the incorporation of salts and/or sugars in the crêping bath. A very suitable salt is, for example, ammonium sulphate, whilst a suitable sugar is ordinary cane sugar.

Having described our invention, what we desire to secure by Letters Patent is:

1. Process for the production of fabrics exhibiting crepe effects, which comprises subjecting a fabric containing high twist yarns of an organic ester of cellulose to over-all saponification to an extent insufficient substantially to affect the dye affinity of said yarns, and thereafter treating the fabric with a creping bath.

2. Process for the production of fabrics exhibiting crepe effects, which comprises subjecting a fabric containing high twist yarns of an organic ester of cellulose to over-all saponification to an extent insufficient substantially to affect the dye affinity of said yarns by means of an aqueous saponifying bath, and thereafter treating the fabric, while it is still wet with the saponifying agent, with a creping bath.

3. Process for the production of fabrics exhibiting crepe effects, which comprises subjecting a fabric containing high twist yarns of an organic ester of cellulose to over-all saponification by treatment with an aqueous saponifying bath followed by drying the fabric while it still contains some saponifying agent, the saponification being

insufficient substantially to affect the dye affinity of the material of the fabric, and after the drying step treating the fabric with a creping bath.

4. Process for the production of fabrics exhibiting crepe effects, which comprises subjecting a fabric containing high twist yarns of an organic ester of cellulose to over-all saponification in an aqueous saponifying bath to an extent insufficient substantially to affect the dye affinity of said yarns, washing the fabric and subjecting it to a creping bath.

5. Process for the production of fabrics exhibiting crepe effects, which comprises subjecting a fabric containing high twist yarns of cellulose acetate to over-all saponification to an extent insufficient substantially to affect the dye affinity of said yarns, and thereafter treating the fabric with a creping bath.

6. Process for the production of fabrics exhibiting crepe effects, which comprises subjecting a fabric containing high twist yarns of cellulose acetate to over-all saponification to an extent insufficient substantially to affect the dye affinity of said yarns by means of an aqueous saponifying bath, and thereafter treating the fabric, while it is still wet with the saponifying agent, with a creping bath.

7. Process for the production of fabrics exhib-

iting crepe effects, which comprises subjecting a fabric containing high twist yarns of cellulose acetate to over-all saponification by treatment with an aqueous saponifying bath followed by drying the fabric while it still contains some saponifying agent, the saponification being insufficient substantially to affect the dye affinity of the material of the fabric, and after the drying step treating the fabric with a creping bath.

8. Process for the production of fabrics exhibiting crepe effects, which comprises subjecting a fabric containing high twist yarns of cellulose acetate to over-all saponification in an aqueous saponifying bath to an extent insufficient substantially to affect the dye affinity of said yarns, washing the fabric and subjecting it to a creping bath.

9. Process for the production of fabrics exhibiting crepe effects, which comprises subjecting a fabric containing high twist yarns of an organic ester of cellulose, to over-all saponification to an extent causing a loss of weight of 1 to 5%, said saponification being insufficient substantially to affect the dye affinity of said yarns, and thereafter treating the fabric with a creping bath.

BERNARD JOSEPH FLANAGAN.  
ALBERT MELLOR.

CERTIFICATE OF CORRECTION.

Patent No. 2,243,858.

June 3, 1941.

BERNARD JOSEPH FLANAGAN, ET AL.

It is hereby certified that error appears in the printed specification of the above numbered patent requiring correction as follows: Page 2, second column, line 2, for "1/2 soap" read --1/2% soap--; and that the said Letters Patent should be read with this correction therein that the same may conform to the record of the case in the Patent Office.

Signed and sealed this 22nd day of July, A. D. 1941.

(Seal)

Henry Van Arsdale,  
Acting Commissioner of Patents.